

March 17, 1925.

1,529,943

A. C. C. M. P. BRUNOT DE ROUVRÉ  
PROCESS FOR OBTAINING METALS HAVING A HIGH MELTING POINT,  
SUCH AS TUNGSTEN  
Filed March 7, 1923



Inventor  
A. C. C. M. P. Brunot de Rouvre  
By *meister Clark*  
Atty.

# UNITED STATES PATENT OFFICE.

ANTOINE CHARLES CONSTANTIN MARIE PHILIPPE BRUNOT DE ROUVE, OF PARIS,  
FRANCE, ASSIGNOR TO SOCIETE ANONYME DES BREVETS BERTHET, OF PARIS,  
FRANCE.

## PROCESS FOR OBTAINING METALS HAVING A HIGH MELTING POINT, SUCH AS TUNGSTEN.

Application filed March 7, 1923. Serial No. 623,514.

To all whom it may concern:

Be it known that I, ANTOINE CHARLES CONSTANTIN MARIE PHILIPPE BRUNOT DE ROUVE, 14 Rue Drouot, Paris, France, have 5 invented Process for Obtaining Metals Having a High Melting Point, Such as Tungsten, of which the following is a full, clear, and exact description.

This invention relates to a process for 10 obtaining metals having a high-melting point; it applies more particularly to tungsten and molybdenum. It allows of obtaining these metals by fusion, thus imparting to them special qualities; more particularly 15 the tungsten obtained by this new process forms a new product which differs much from the tungsten which is manufactured according to the known method.

Up to now, it has been impossible to obtain 20 molten tungsten because if a carbon crucible is used, tungsten carbide is formed and if other substances are used for making the crucible, the latter is destroyed before the tungsten melts.

25 The process which is the object of the present invention does away with these two serious drawbacks. It consists essentially in causing an electric arc to strike in a gaseous medium, between two electrodes made 30 of tungsten (for instance) and in causing tungsten powder to fall gradually upon the crater of the arc (or even upon one only, which will preferably be the positive crater when the arc is fed by a direct current).

35 When the current of the electric arc is adjusted in a suitable manner, the crater of the electrodes melts superficially and the tungsten powder melts gradually according 40 as it falls upon this crater; by continuing with this operation, the volume of the electrode is little by little increased by a deposit of molten tungsten. Hydrogen is suitable as the surrounding gas in this case; however, hydrogen may be simultaneously 45 used with a nitrogen and with another gas having the same properties.

The use of several gases may be necessary for the purification of the tungsten because the powder which is found in the trade 50 often contains foreign substances.

Instead of metallic powder, an oxygenated compound of the metal (for instance,

tungstic acid) may be used, when the surrounding gas contains hydrogen.

An apparatus enabling the carrying of 55 the process according to the present invention into effect, will be hereinafter described, by way of example. With reference to the accompanying drawing, in which the figure is a diagram of the apparatus, 60

This apparatus comprises two vertical electrodes *a* and *b*; the upper electrode *b* is pierced by a small axial channel *c* through which passes the powder to be melted. A distributor, consisting for instance of a small Archimedean screw *d*, takes the tungsten powder into a receptacle *e* provided to this end and brings it above the orifice of the channel of the upper electrode; this powder falls little by little upon 70 the crater of the lower electrode *a* and melts as it has been explained above. In order to ensure a complete and regular fusion upon the entire surface of the lower electrode, the latter may be displaced in a horizontal 75 plane; in this manner the arc may be successively brought upon all the points of the electrode.

According as the tungsten increases the 80 length of the lower electrode, the latter is moved away in such a manner that the arc shall always have the desired length. All 85 these arrangements may be rendered automatic by means of an electric or mechanical drive which is easy to establish, such as a small motor *f*, causing the rotations by means of a tangent screw *g* of the lower electrode and actuating by means of a relay *h*, an arrangement intended to move the electrodes apart and to proportion the 90 delivery of the powder to the speed of fusion.

The tungsten powder may also be brought 95 to the arc by means which are independent of the electric circuit; in this case the arc may be struck by means of any known arrangement of electrodes.

When a molten mass has been obtained, the latter is subjected to a hammering which imparts to it a shape suitable for the purpose for which it is intended, permitting for 100 instance its passing through drawing plates for the purpose of obtaining filaments for electric arcs. The hammering and the wire drawing may be carried out with heat in an

indifferent or reducing medium. These filaments may be advantageously used in electric vacuum or gas lamps and give better results than the filaments which have been hitherto used.

It is also possible to hammer and to roll the ingot for obtaining plates.

Owing to the qualities obtained by fusion, the tungsten thus obtained can be much 10 more easily worked than the tungsten worked by the known methods.

Claims:

1. A process for obtaining by melting metals having a very high melting point, 15 such as tungsten, which consists: in gradually pouring, in a pulverulent condition, the metal to be melted in the crater of an electric arc struck, in a non-oxydizing atmosphere, between two electrodes made of metal 20 the melting point of which is equal or superior to that of the metallic powder to be melted, in regulating the fall of the said metallic powder in such a manner that the latter melts in proportion to its arrival in 25 the crater of the electric arc and becomes soldered to the electrode presenting this crater and that this electrode thus increases progressively in size by the successive deposits of molten metal, and in constantly 30 regulating the spacing apart of the electrodes in proportion to the deposits of molten metal so that the electric arc may always have the same length.

2. A process for the manufacture of small 35 sticks of molten tungsten which consists: in gradually pouring tungsten powder in the crater of an electric arc struck in a non-oxydizing atmosphere, between two elec-

trodes made of tungsten, in regulating the fall of this tungsten powder so that the latter melts in proportion to its arrival in the crater of the electric arc and becomes soldered to the electrode presenting this crater, and that this electrode thus increases progressively in size by the successive deposits of molten metal, and in constantly regulating the spacing apart of the electrodes in proportion to the said deposits so that the electric arc may always have the same length.

3. A process for obtaining by melting metal having a very high melting point, such as tungsten, which consists: in gradually pouring, in a pulverulent condition, the metal to be melted in the craters of electric arcs struck between several electrodes made of a metal the melting point of which is equal or superior to that of the metallic powder to be melted, in regulating the fall of the said metallic powder in such a manner that the latter melts in proportion to its arrival in the craters of the electric arcs and becomes soldered to the electrodes presenting these craters, and that these electrodes thus increase progressively in size by the successive deposits of molten metal, and in constantly regulating the spacing apart of the electrodes in proportion to the said deposits so that the electric arcs may always have the required length.

The foregoing specification of my "Process for obtaining metals having a high melting point, such as tungsten" signed by me this 23d day of February 1923.

ANTOINE CHARLES CONSTANTIN MARIE PHILIPPE  
BRUNOT DE ROUVRE.